

July 1, 1930.

S. D. WELLS

1,769,811

PROCESS OF PULPING FIBROUS MATERIAL

Filed Nov. 7, 1928

Fig. 1.



Fig. 2.



Inventor  
Sidney D. Wells  
By W. L. Symons  
his Attorney

## UNITED STATES PATENT OFFICE

SIDNEY D. WELLS, OF QUINCY, ILLINOIS, ASSIGNOR, BY MESNE ASSIGNMENTS, TO THE MINE & SMELTER SUPPLY COMPANY, OF DENVER, COLORADO, A CORPORATION OF COLORADO

## PROCESS OF PULPING FIBROUS MATERIAL

Application filed November 7, 1928. Serial No. 317,704.

This invention relates to a process of pulping fibrous vegetable material and pertains particularly to the treatment of straw and other fibrous vegetable material with caustic alkali solutions at low temperatures.

5 An object of this invention is to effect lignin removal with as little loss as possible of cellulose and pentosans.

In all cooking processes for separating the fibers of straw and other fibrous vegetable 10 material, the pulping agents should act upon the lignin to the greatest extent to bring about the most effective softening or solution of the incrusting constituents. The processes commonly used do so only with the dissolution 15 and loss of considerable cellulose and pentosans.

Attempts have been made to diminish this loss by the use of reducing substances such as sulphides, sulphites, and so forth, in conjunction 20 with the cooking lyes.

In accordance with the present invention, it has been found that excellent results are obtained by soaking the fibrous material, such 25 as straw or esparto, in solutions of caustic soda or potash at temperatures below 100° C. before disintegration of the material. By the term "cold" herein is meant temperatures below 100° C. in contrast with the higher or 30 cooking temperatures in ordinary use.

The following table indicates the relative efficiency of typical cooking processes and the present caustic alkali process at room temperature, namely, about 25° C.

|                                               | Pento-sans and cel-lulose | Lignins  | Loss of cel-lulose and pento-sans | Lignin re-moved |
|-----------------------------------------------|---------------------------|----------|-----------------------------------|-----------------|
|                                               | Per cent                  | Per cent | Per cent                          | Per cent        |
| 40 Composition of straw before treatment      | 64.7                      | 24.1     |                                   |                 |
| 45 Composition of fiber after treatment with: |                           |          |                                   |                 |
| Lime                                          | 47.5                      | 12.9     | 17.2                              | 11.3            |
| Caustic soda—                                 |                           |          |                                   |                 |
| At 150° C.                                    | 46.4                      | 5.3      | 18.3                              | 18.8            |
| At 100° C.                                    | 46.6                      | 7.3      | 18.1                              | 16.8            |
| Soda ash and sulphite                         | 50.4                      | 16.4     | 14.3                              | 7.7             |
| Caustic soda at 25° C.                        | 60.5                      | 10.2     | 4.2                               | 13.9            |

In the above table, it is noted that the cellulose and pentosans lost, are considerably

less in the cold process and that the latter process compares favorably with the other processes in the amount of lignin removed.

In the accompanying drawing, Figures 1 and 2 are diagrammatic representations of the apparatus which may be used to carry out the process of this invention.

For carrying out the process of the present invention, it is preferable to employ a counter-current method of soaking the fibrous material treated. For instance, as shown diagrammatically in the accompanying drawing, Figure 1, there may be five sets of tanks numbered I, II, III, IV, and V connected in any suitable fashion by pipe lines as indicated.

At a given time, one set of tanks is being filled, another set has had the fibrous material in soak for three days and is being emptied, and the other three sets have had the straw in soak approximately one, two and three days respectively.

For example: Set I is being filled with straw and the straw in set V is finished and is removed to the mill for beating, washing, and manufacturing into paper. The straw in set II is completing its first day of soaking with liquor taken from set III and what is squeezed from the straw removed from set V. The straw in set III has completed its first day of soaking in set II and is completing its second day of soaking in liquor taken from set IV. The straw in set IV has completed its first and second days of soaking in sets II and III respectively and is completing its third day of soaking in fresh liquor.

Starting with fresh liquor containing about 15 grams of caustic soda per liter, after the first day of soaking in set IV, the concentration of the liquor is reduced to about 10 grams of active caustic soda per liter. At the end of the soaking in set III the concentration of the liquor is about 6 grams per liter, and at the end of the soaking in set II from whence the liquor is passed to waste or treated for the recovery of alkali, the concentration is about 3 grams of caustic soda per liter.

When the straw is removed from set IV into set V, it is saturated with liquor in which there is much free caustic alkali. Much of this liquor may be squeezed out and used

earlier in the soaking process. For instance, about five tons of liquor are required to immerse one ton of straw. When the straw is removed from the liquor in a given tank, 5 about two tons of liquor are held in each ton of the straw. Starting with dry straw in tank II it will be seen that only three-fifths of the required quantity of liquor is available from tank III. The other two-fifths are therefore 10 obtained for tank II by squeezing out of the wringing wet straw from tank V by means of squeeze rolls as shown in the diagram. The straw may be then washed out and the strongest of the wash waters used earlier in the 15 soaking process.

Alternatively, the straw from tank V may be passed through a rod mill and the liquor removed by a dewatering or washing device after the straw has been properly pulped. 20 The rod mill or other beating device is operated between room temperature and 100° C. at atmospheric pressure. No pressure is permitted to develop in the rod mill and it is preferable to blow in as much steam as will 25 con dense without developing pressure. A temperature of about 90° C. is thus obtained. As much as possible of the unconsumed alkali present in the straw is utilized by employing heat in the rod mill during the pulping operation. 30

The pulped material from the rod mill is washed and the strongest of the wash liquors used in the first step of the soaking process. A suitable rod mill for performing this 35 operation is shown in my Patent, No. 1,654,624, issued January 3, 1928.

Instead of the series of tanks represented by Fig. 1, an apparatus such as that diagrammatically shown in Fig. 2 may be used, in the 40 form of a long trough with straw fed in at one end and liquor at the other. The straw is carried slowly through the trough by means of some suitable conveying or raking device.

It is sometimes desirable to subject the material to a digestion treatment after the soaking treatment. In this case, the soaking treatment would be carried on for the purpose of delignifying to the extent that it is profitable to go in the cold. Further delignification would be accomplished by digestion of the material in the liquor which it encountered after removal from the soaking treatment and at elevated temperatures up to 100° C. The second delignification results in a 55 greater loss of pentosans and cellulose than was encountered in the soaking treatment, but the total loss in both treatments is much less than in digestion at elevated temperatures as commonly practiced.

60 By the process of this invention, a more uniform product is obtained than is obtained in the ordinary processes in common use and this with a maximum amount of disintegration and with the least consumption of power.

65 The quality of the product is improved be-

cause the fibers separate into intact units without rupture on account of the complete soaking it has had before the disintegration operation.

What I claim is:—

1. A process of separating the fibers of fibrous vegetable material, which process comprises soaking the fibrous material in a cold caustic alkali solution, and subjecting the soaked material to treatment in a rod 75 mill.

2. A process of separating the fibers of fibrous vegetable material, which process comprises soaking the fibrous material in a cold caustic alkali solution, and treating the 80 soaked material to steam in a rod mill.

3. A process of separating the fibers of fibrous vegetable material, which process comprises soaking the fibrous material in a cold caustic alkali solution, and treating the 85 soaked material with steam in a rod mill at atmospheric pressure.

4. A process of separating the fibers of fibrous vegetable material, which process comprises soaking the fibrous material in a cold caustic alkali solution, and treating the 90 soaked material with steam in a rod mill at atmospheric pressure below 100° C. to utilize the alkali left in the straw from the soaking step.

5. A process of separating the fibers of fibrous vegetable material, which process comprises soaking the fibrous material in a caustic alkali solution at a temperature below 100° C., and subjecting the soaked material 100 to treatment in a rod mill.

In testimony whereof I affix my signature.

SIDNEY D. WELLS.

105

110

115

120

125